

July 17, 1923.

1,461,862

W. R. CLARK

MANUFACTURE OF ELECTRIC FURNACE LININGS

Filed Aug. 6, 1917

Fig. 1.



Fig. 2.



Fig. 3.



Fig. 5.



Fig. 4.



INVENTOR  
Walter R. Clark,  
BY *Alvin M. MATTISON*

## UNITED STATES PATENT OFFICE.

WALTER R. CLARK, OF BRIDGEPORT, CONNECTICUT, ASSIGNOR TO BRIDGEPORT BRASS COMPANY, OF BRIDGEPORT, CONNECTICUT, A CORPORATION OF CONNECTICUT.

## MANUFACTURE OF ELECTRIC-FURNACE LININGS.

Application filed August 6, 1917. Serial No. 184,675.

*To all whom it may concern:*

Be it known that I, WALTER R. CLARK, a citizen of the United States, residing in Bridgeport, in the county of Fairfield and 5 State of Connecticut, have invented certain new and useful Improvements in the Manufacture of Electric-Furnace Linings, of which the following is a full, clear, and exact description.

10 This invention relates to the manufacture of electric furnace linings, and more particularly the linings of induction furnaces of the type in which a tube or passage of closed cross-section, communicating with 15 the hearth at two points, receives a portion of the molten bath, which acts as the secondary of the transformer. The molten metal is circulated through the secondary passage or channel by "motor effect", there- 20 by establishing a circulation of the bath and transmitting the heat to all portions thereof. The channel, tube or passage through which the metal of the secondary flows is usually formed of, or lined with a suitable 25 material which will satisfactorily withstand the high temperature developed.

In furnaces of the type mentioned, especially where the secondary is of rather small cross-section, it is very difficult to form the 30 refractory portion having, or associated with, the secondary passage, channel or duct, in such a way that the wall of the passage or duct will be perfectly homogeneous, and at the same time, sufficiently smooth, and 35 uniform in cross-section, for proper furnace operation. One of the methods heretofore used in making the refractory structure having the secondary passage, channel, duct or bore was to ram up a furnace 40 lining around a casting composed of an alloy of the materials which were to be melted in the furnace later on. Such an alloy casting is of the same cross-sectional area and shape as the desired secondary channel of 45 the furnace and serves as a pattern or tem- 50 plet around which the refractory material is rammed, the templet or pattern being held meantime in a suitable frame. After the furnace has been completed by the ad- 55 dition of further refractory material for forming the hearth, and after the entire structure has been properly dried, the alloy pattern is melted by making the necessary electrical connections. Additional metal is introduced into the furnace in the molten

state to increase the volume of the molten bath, so that it will act as a bed for receiving the first charge to be melted. In this way, the pattern is utilized to create a portion of the bath when the completed fur- 60 nace is first placed in operation.

In furnaces constructed in this manner, especially when used for melting materials having fairly high melting points, for example, brass scraps or turnings, the expansion of the metal pattern or templet which is incident to heating it to the melting point, is considerable, because in such case, the pattern or templet is made of the same material, e. g., brass, which is to be melted 65 in the furnace. Owing to the shape of the pattern, its considerable expansion prior to melting, creates great pressure upon the surrounding lining, which usually has a different coefficient of expansion. This pressure is so great as to frequently cause small 70 cracks or fissures to appear in the refractory lining, which will cause the same to have a very short life, sometimes causing failure of the furnace from the start, due to the leak- 75 age of the molten metal through these cracks or fissures. This destructive pressure of the pattern may be exerted in a lateral direction relatively to the secondary channel, or in a longitudinal direction rela- 80 tively thereto, or in both directions, or in any one or more oblique directions. Of course the longitudinally exerted pressure is detrimental owing to the very close frictional contact between the pattern and the 85 lining. During the preliminary heating op- 90 eration, the stress put upon the pattern is sometimes sufficient to cause a complete rup- 95 ture of the same, thereby creating a gap in the secondary circuit, which it is impossible to close, making it necessary to pull down and rebuild the furnace. Such rupture of the pattern is especially liable to occur in the melting of brass because a brass pat- 100 tern will often become more or less brittle at some temperature between the ordinary atmospheric temperature and the ordinary melting point, depending upon the composition thereof; and under such conditions the lengthening or extension of the pat- 105 tern caused by the heat applied in the preliminary heating frequently causes it to break in two.

Patterns have been made of wood, and the same have been burned out after the ram-

65

70

75

80

85

90

95

100

105

110

ming and drying operation is completed, but this procedure is very slow and unsatisfactory, and it is very difficult to remove the wood entirely from any sharp corners of the secondary passage should the latter be made with one or more sharp turns, as is frequently the case.

The primary object of my present invention is to obviate the above mentioned difficulties and to facilitate the manufacture of induction furnaces of the type above described. Another object of the invention is the provision of a pattern for the purpose indicated, which neither injuriously affects the lining of the furnace, nor the metal or alloys which the furnace is intended to melt, which pattern is hard enough and strong enough at ordinary temperatures to allow the refractory to be rammed about it in a satisfactory way, but which, nevertheless, does not exert injurious pressure on the lining during the preliminary melting.

To these and other ends, the invention consists in the novel features and procedure hereinafter described and claimed.

In the accompanying drawing,

Fig. 1 is a vertical central section of an induction furnace, showing the same in the process of construction, with a reinforced wax templet or pattern in the secondary channel;

Fig. 2 is a detail of the templet or pattern shown in Fig. 1;

Fig. 3 is a side elevation of the templet; Fig. 4 is a section on line 4—4 of Fig. 1; and

Fig. 5 is a cross-section of another templet which may be employed.

In the drawing, I have shown an electric induction furnace having a body 10, composed of a metal jacket or casing 11, and a refractory lining 14. The furnace has a basin or hearth 13 at the upper part, which in this case is formed in a layer or body of refractory material packed within a layer 12 of suitable heat insulating material, such for example as infusorial earth. The layer 14 advantageously consists of a suitable asbestos cement, although I do not limit myself in this respect. The hearth has a pouring spout 15, and a charging opening 16, having a door 17. Beneath the hearth of the furnace shown herein is a closed channel of approximately V-shape, indicated at 18, having substantially straight side portions communicating with each other at an acute angle, as shown at 19, and connecting with the hearth at opposite sides of the latter, as shown at 20. The metal which is received in the channel 18 in the operation of the furnace acts as a secondary of a transformer whose primary is constituted by a horizontally arranged core 21 extending about the upper portion of the channel 18 and having a winding 21<sup>a</sup> suitably con-

nected with a source of current. Owing to the arrangement of the two legs of the channel 18 at an acute angle to each other, the action of the primary is such as to set up a thorough circulation of molten metal in the channel and the bath or pool in the hearth, it being understood, of course, that in practice the upper ends of the continuous channel are in constant communication with the lower part of the hearth which is filled to approximately the level of the pouring spout with a bath of molten metal.

In constructing the lower portion of a furnace such as that selected for illustration, I use a pattern or templet 22 for forming the channel 18 in the refractory material. This pattern or templet 22 is of the same shape as the passage or channel, which it is desired to form, and in the embodiment shown in Figs. 1-4, it consists of a body 23 of a paraffine, or other hydrocarbon or the like, in which is embedded a metallic core 24 which may advantageously consist of woven copper wire in the form of a sheet which is embedded in the center of the paraffine. This pattern or templet 22 is held in position in a suitable frame, and the refractory material, such as asbestos, cement, in which the secondary channel is to be formed, is tamped around the pattern. The paraffine or so called paraffine wax is sufficiently hard and strong at ordinary temperatures to allow the refractory material to be firmly packed or rammed around it, so as to obtain a channel of uniform cross-section having a smooth, homogeneous surface. The structure is then dried. It may be dried in a suitable oven or kiln, for example, and when so dried, the heat is sufficient to melt the paraffine and to cause it either to flow into and fill the minute voids of the lining or to flow out of the channel. Or, if desired, the refractory material can be dried electrically by passing an electric current through the metallic core 24, which melts the paraffine and usually drives it into the lining, at the same time that the heat generated by the current dries out the lining. In drying out the lining electrically the ends of the metal portion of the templet 22 may be connected to the poles of an exterior source of current, or the transformer may be utilized if the metal portion of the templet is suitably short circuited so that it will form a closed circuit, for example, by interconnecting the ends of the metal with a piece of wire. This wire is removed after the furnace has dried, for, in starting the furnace, molten metal poured into the hearth will complete the secondary in an obvious manner. The paraffine has no deleterious effect upon the lining nor upon the metal or alloys which are to be melted. The driving of the solid hydrocarbon into the voids of the lining is a feature of ad-

vantage by reason of the fact that the substance in question carbonizes and thus fills up the voids and increases the density of the lining; and, as will be obvious, it also 5 provides an easy way of disposing of the non-metallic portion of the pattern preliminary to the actual use of the furnace. In the case now being considered, the metallic reticulated or foraminous material 10 remains in the channel after the paraffine has been eliminated, and the radiation of heat from the metallic conductor therein can then be continued by maintaining the electrical connections, so as to thoroughly dry 15 out said passage. The metal portion of the pattern may also remain in the channel when the furnace is placed in operation, inasmuch as it will, if made of suitable material, alloy properly with the material 20 to be melted in the furnace. If brass, for example, is to be melted in the furnace, the reticulated core of the pattern may either be made of brass or copper.

It is important to note that in starting 25 the furnace after the paraffine has been driven out of the channel and the refractory has been properly dried, the metal remnant of the pattern is not in tight contact with the wall of the channel. By 30 making the core of suitable reticulated material, it is extensible to a considerable degree without breaking, and even if a fairly high temperature is necessary to melt it, it will not rupture before melting, and 35 therefore the secondary is not likely to be broken or interrupted. The metallic core or other remnant, in expanding, does not exert on the lining any such pressure as would injuriously affect it. I consider it 40 most advantageous to make the metallic core of a fabric woven from copper wire, as copper is ductile at all temperatures up to melting, and in case the furnace is started on brass (with molten brass poured in 45 around the core), and the brass tends to solidify in the secondary passage, the ductility of the wire will usually prevent effectively a complete or harmful rupture of the secondary.

50 If, under certain circumstances, it is desired to prevent the paraffine from being driven into the lining material, when the former is melted, the paraffine templet may be coated on the outside with shellac or 55 varnish of high melting point. This will enable the melted paraffine to be poured out of the channel without going into the lining.

In other cases, I may use a pattern comprising a very thin metal tube of the metal 60 which is to be melted in the furnace, the said tube being filled with wax, sand, or other suitable substance, which reinforces it interiorly to such an extent as to offer sufficient resistance to ramming. In Fig. 65 1, I have shown in cross-section a thin metal

tube 25, which may be of copper, for example, and in the tube is a filling 26 of sand, which prevents the tube from collapsing when the refractory material is rammed about it. When the operation of ramming 70 is completed, the sand can be run out of the tube very readily, as will be understood.

In heating up the refractory structure, either for drying it or in starting the furnace, and either by the application of external heat, or by the use of an electric current passing through the metallic tubular core, the tube will collapse inwardly in a lateral direction under the expanding influence of the heat instead of expanding laterally in an outward direction, or extending itself lengthwise, and hence there will be no severe lateral and outward pressure, or oblique pressure, or longitudinal pressure on the lining, or, at any rate, not sufficient pressure in any of those directions to crack the lining or affect it injuriously. If the tubular pattern is filled with wax, for example, the wax can be quickly eliminated by passing a current through the tube, which is thereby permitted to collapse inwardly. In other words, as the wax is quickly eliminated, it offers no appreciable resistance to the inward collapse of the tube, and outward pressure is thereby prevented. In case the tube is filled with sand, the latter is of course poured out before the tube is heated so as to permit the inward collapse of the tube. The tube can be utilized in starting the furnace in substantially the same manner as the other metallic templet remnant hereinbefore described.

A tube such as that shown in Fig. 5, may not only be made of copper or other metal of low melting point, but it may be made of metals having a high melting point, such as platinum, tungsten alloy, or nickel chrome alloy, where certain materials are to be melted in the furnace. Tubes of high melting point will hardly be used, however, except 105 in rather exceptional cases.

Various changes may be made in the procedure and apparatus herein particularly described without departing from the scope of my invention as defined in the claims.

I do not claim specifically herein a templet for the manufacture of electric induction furnaces and the like, having an interior filling of readily meltable material, as claimed in my divisional application Serial No. 322,556.

What I claim is:—

1. The method of making the refractory structure of an electric furnace or the like having an interior passage or channel, which comprises tamping refractory material about a pattern of the same shape as the passage to be formed, made at least partly of a non-metallic material which at ordinary temperatures is sufficiently hard and strong to

resist collapse under the tamping pressure, but which melts at a low temperature, and applying heat to the structure for removing such non-metallic material from the passage, 5 and drying the structure.

2. The method of making the refractory structure of an electric induction furnace having a passage of closed cross-section arranged beneath and in communication with 10 the hearth or basin thereof, which comprises tamping refractory material on all sides but not at the ends about a pattern of the same shape as the passage to be formed, and which is made at least partly of a pliable, 15 readily meltable, non-metallic solid which is sufficiently hard and strong to resist distortion under the proper tamping pressure, and then melting such material by the application of heat.

20 3. The method of making the refractory structure of an electric induction furnace having a passage of closed cross-section arranged beneath and in communication with the hearth or basin thereof, which comprises 25 tamping refractory material at different sides but not at the ends about a pattern of the same shape as the passage to be formed and which is made at least partly of a pliable, readily meltable, non-metallic solid 30 which is sufficiently hard and strong to resist distortion under the proper tamping pressure, then melting such material by the application of heat and running off a portion of the same from the passage ends, and 35 continuing the application of heat after the melting of such material to dry the refractory material thoroughly.

4. The method of making the refractory structure of an electric furnace or the like 40 having an interior passage, which comprises tamping the refractory material about a pattern or templet which consists partly of a metal conductor and partly of a body of material of a lower melting point than said 45 conductor, melting and thereby eliminating the low melting point portion of the pattern after the tamping operation has been completed, and then drying the structure while the metallic conductor portion of the pattern 50 remains in place.

5. The method of making the refractory structure of an electric furnace or the like having an interior passage of closed cross-section, which comprises tamping the refractory material about a pattern or templet 55 which is made partly of metal of high melting point and partly of a body of low melting point, eliminating the low melting point portion of the pattern by melting after the 60 tamping operation has been completed, and then drying the structure.

6. The method of making the refractory structure of an electric induction furnace having a passage of closed cross-section arranged beneath and in communication at

both ends with the hearth or basin thereof, which comprises tamping plastic refractory material on all sides of a pattern of the same shape as the passage to be formed, but leaving such pattern free at the ends, such pattern consisting at least partly of a pliable, readily meltable solid, then melting such material so that a portion thereof is absorbed by the lining of the passage and then carbonizing the material so absorbed by the lining. 70

7. The method of making a refractory structure of an electric induction furnace having a secondary passage, which comprises supporting in a suitable frame, a pattern of the same shape as the secondary passage to be formed, such pattern consisting at least partly of a non-metallic material which at ordinary temperatures is sufficiently hard to resist collapse under tamping pressure but which melts at a low temperature, tamping refractory material in plastic condition about the sides of such pattern, but leaving the same free at one or more points to permit the escape of the melted material, applying heat to the structure for melting and eliminating such material, and continuing the heating of the structure so as to dry the same and carbonize any of the pattern material absorbed in the lining of the passage. 80

8. The method of making an electric induction furnace and placing it in operation, which comprises ramming refractory material about a pattern composed partly of metal and partly of a substance of low melting point, eliminating by melting the low-melting point substance and drying the furnace structure, passing an electric current through the metallic remnant of the pattern when the furnace is to be placed in operation, and pouring into the furnace molten metal which makes contact with the metallic remnant of the pattern while the current traverses the latter. 90

9. The method of lining the hearths of electric induction furnaces, which comprises placing the lining material around a templet consisting partly of metal and partly of a thick coherent non-metallic unitary body of low melting point which is sufficiently hard to withstand the ramming pressure at ordinary temperatures, eliminating by melting the non-metallic body after the lining material has been tamped in place, pouring molten metal into the furnace around the remnant of the templet, and passing electric current through such metallic remnant, for starting the furnace. 100

10. The method of making the refractory structure of an electric induction furnace, which comprises ramming refractory material around a templet composed partly of wax and partly of metal, heating the wax to melt and eliminate the same, pouring molten metal into contact with the metallic 110 115 120 125 130

remnant of the templet, and passing electric current through such metallic remnant, for starting the furnace.

11. The method of making the refractory structure of an electric induction furnace having a secondary passage of closed cross-section arranged beneath and in communication with the hearth or basin thereof, which comprises tamping refractory material on all sides, but not at the ends, about a pattern of the same shape as the passage to be formed and which consists partly of metal and partly of non-metallic material of low melting point, eliminating the non-metallic portion of the pattern by melting the same after the tamping operation has been completed, and then drying the structure while the metallic portion of the pattern remains in place.
12. The method of making and operating an electric induction furnace having a secondary passage of closed cross-section arranged beneath and in communication with the hearth or basin thereof, which comprises tamping refractory material on all sides, but not at the ends, about a pattern of the same shape as the passage to be formed, which pattern consists partly of non-metallic material of low melting point and partly of an interior metal reinforce, melting and thereby eliminating the non-metallic portion of the pattern after the tamping operation has been completed, and operating the furnace while the metallic portion of the pattern remains in place in the passage.

13. The method of making an electric induction furnace having a hearth with a heating passage connected therewith, which comprises ramming refractory material about a templet of the same shape as the passage to be formed, said templet consisting of a readily meltalbe non-metallic body having a metallic core extending from one end of the templet to the other, eliminating the non-metallic component of the templet by the application of heat, passing an electric current through the core after the non-metallic component has been eliminated, and starting the furnace while such electric current traverses the core.

14. The method of constructing and operating an electric induction furnace having a hearth or chamber with a secondary passage of closed cross-section connected therewith, which comprises ramming suitable plastic material about a templet of the same shape as the passage to be formed, said templet consisting partly of metal and partly of a non-metallic substance of low melting point, then eliminating by melting the non-metallic portion of the templet, and melting the metallic remnant of the templet when the furnace is to be started.

15. The method of constructing and op-

erating an electric induction furnace having a chamber with a secondary passage of closed cross-section connected therewith, which comprises ramming a suitable plastic material about a templet of the same shape as the passage to be formed, and consisting partly of metal and partly of a readily meltalbe non-metallic substance, applying heat to the structure for melting and eliminating the non-metallic component of the templet, inducing an electric current in the metallic remnant of the templet to melt the same in said passage, and placing additional metal in the furnace chamber to complete the charge.

16. The method of constructing and operating an electric induction furnace having a secondary passage, which comprises ramming a suitable plastic material about a templet of the same shape as the passage to be formed, said templet consisting partly of a metal conductor and partly of material of lower melting point than said conductor, melting out the material of lower melting point, and melting the metallic conductor portion of the templet in said passage when the operation of the furnace is commenced.

17. The method of making and operating an electric induction furnace having a secondary passage, which comprises tamping about a pattern or templet of the same shape as the secondary passage to be formed, refractory material, such pattern or templet consisting of a metallic inner part and a readily meltalbe non-metallic outer part, melting the non-metallic outer part of the pattern to eliminate the same after the tamping operation has been completed, and starting the furnace while the metallic portion of the pattern remains in place in the secondary passage.

18. In the manufacture of an electric induction furnace having a refractory structure with a secondary passage therein, increasing the density of the lining of such passage by treatment with a non-metallic material which closes the pores of the refractory.

19. In the manufacture of an electric induction furnace having a refractory structure with a secondary passage therein, the step of treating the lining of the passage with a hydrocarbon.

20. In the manufacture of an electric induction furnace having a refractory structure with a secondary passage therein, treating the lining of the secondary passage with material containing a hydrocarbon, and then carbonizing such material, whereby the density of the lining is increased.

21. In the manufacture of a refractory furnace structure having an interior passage, driving a waxy substance into the lining of the passage by the application of heat.

22. The method of making the refractory structure of an electric furnace having an interior passage, which comprises tamping the refractory material about a pattern or 5 templet, which consists of an outer waxy body of considerable bulk and an inner flexible metallic conductor, melting the waxy portion of the pattern so as to drive at least a part of the waxy material into 10 the lining of the passage to thereby improve the same, and drying the structure while the metallic portion of the pattern remains in place.

23. In the manufacture of a refractory 15 furnace structure, the step of filling up the voids in the refractory by treatment with a waxy substance.

24. In the manufacture of a refractory furnace structure, the step of filling up the 20 voids in the refractory by treatment with a waxy substance, which is subsequently carbonized.

25. A templet for the purpose described 25 consisting partly of wax and partly of a flexible copper reinforce embedded in the wax and extending out of the same at both ends of the templet.

26. A templet for the purpose described, 30 consisting partly of wax and partly of a longitudinal reinforce embedded in the wax, such reinforce comprising one or more strands of ductile metal.

27. A templet for the purpose described, 35 which comprises a wax-like body having a reticulated flexible reinforce embedded therein and extending longitudinally therethrough.

28. A templet such as described having a 40 metallic core extending longitudinally therethrough.

29. A templet for the purpose described, having a reticulated copper core embedded 45 therein and extending therethrough.

30. The method of starting an induction 45 furnace, which consists in placing within the heating space of said furnace a composite body formed of materials of different melting points, then melting the material of lower melting point, and then melting 50 the material of higher melting point.

31. The method of starting an induction furnace, which consists in placing within the heating space of said furnace a composite body formed of materials of different melting 55 points, then melting the material of lower melting point, and then melting the material of higher melting point by induction.

32. The method of starting an induction 60 furnace, which consists in placing within the heating space of said furnace fusible materials of different melting points respectively, then melting the material of lower melting point, and finally melting the

material of higher melting point, whereby 65 the lateral pressure against the refractory wall is minimized.

33. The method of making the refractory structure of an electric furnace, which comprises placing within the furnace space a 70 composite body formed of materials of high and low melting points respectively, melting the low melting point portion of the body, drying the structure, and then utilizing the high melting point portion of the body for 75 starting the furnace, by inducing a current therein.

34. The method of making and operating an induction furnace, which comprises placing 80 in a refractory furnace structure a composite body having portions of different melting points adapted for successive melting in placing the furnace in operation, so as to minimize the lateral pressure on the refractory wall.

35. The method of making an electric furnace, which comprises building a refractory structure about a composite templet composed of a conductor portion of high melting point and a portion of low melting point, one of said templet portions being 90 located at a substantial distance from the lateral walls of the refractory structure, and inducing a current in the templet to fuse the portion of low melting point.

36. The method of drying a green refractory structure, which comprises the location 95 of a composite electric conductor within but at a substantial distance from the lateral walls of the refractory body, and the induction of current in said conductor, whereby the pressure on such lateral walls is minimized.

37. The method of making an electric furnace, which comprises building a refractory 100 structure about a composite conductor templet composed of a portion of high melting point and a surrounding thick unitary body of low melting point, inducing a current 105 in the templet to fuse and eliminate the portion of low melting point, and continuing the induction for drying out the furnace.

38. The method of making an electric furnace, which comprises building a refractory structure about a composite conductor templet composed of a portion of high melting point and a thick solid body of low melting point, inducing a current in the templet to fuse and eliminate the portion of 110 low melting point, and continuing the induction for drying out the furnace, and finally, melting the portion of high melting point for starting the furnace.

In witness whereof, I have hereunto set 115 my hand, on the 2nd day of August, 1917.

WALTER R. CLARK.